

1

3,434,838  
**HEAT-DEVELOPABLE REPRODUCTION  
MATERIAL**

Johannes Munder and Günther Hertzberg, Wiesbaden-Biebrich, Germany, assignors, by mesne assignments, to Keuffel & Esser Company, Hoboken, N.J.

No Drawing, Filed Feb. 24, 1965, Ser. No. 435,027  
Claims priority, application Germany, Feb. 29, 1964,

K 52,254

Int. Cl. G03c 1/58

U.S. Cl. 96—75

8 Claims 10

## ABSTRACT OF THE DISCLOSURE

A heat-developable diazotype reproduction material is prepared by impregnating, during the paper-making process, a paper carrier sheet with a heat-active source of alkaline material, such as urea. Upon completion of the paper-making process, the impregnated paper sheet is coated with a composition including a light-sensitive diazonium compound and a coupler compound capable of forming an azo dye with such diazonium compound in an alkaline medium. Heating of the resulting sheet material creates an alkaline medium conducive to the coupling reaction between the diazonium and the azo coupler compounds and effects development of an azo dye.

The present invention relates to reproduction materials and refers more particularly to a heat-developable two-component diazotype reproduction material.

For the preparation of photocopies according to the diazotype copying process, two methods are used: the dry process and the semi-wet process. In the dry process, the copying material includes a diazo compound and an azo coupling component, and development is effected with ammonia gas. In the semi-wet process, the copying material includes a diazo compound and development is effected in acid or alkaline solution with an azo coupling component to form an azo dye in the unexposed areas.

One disadvantage in the conventional development of such photocopies is the unpleasant odor caused by the ammonia used in the dry process and the inconvenient use of a liquid bath in the semi-wet process. Consequently, since the introduction of the diazotype process, attempts have been made in the art to initiate dye formation by the action of steam or heat.

The coupling process with phenols proceeds smoothly only in alkaline to neutral pH-range. Accordingly, prior attempts were directed to a pH shift by temperature increase with the optional use of suitable additives. This pH shift can be achieved by removal of a volatile acid or by generating alkaline substances from non-alkaline substances. Additives causing the pH shift were generally applied in special coatings between the light-sensitive composition and the support of the coating, or to the side away from the light-sensitive coating. One disadvantage is the deleterious effect on the shelf life of the copying material or the impaired quality of the copies produced.

Therefore, one object of the present invention is to provide a heat-developable, two-component diazotype reproduction material which overcomes these disadvantages.

Another object is to provide a heat-developable reproduction material having excellent shelf life with excellent quality in the photocopies produced therefrom.

Other objects will be apparent in the course of the following specification.

The object of the present invention may be realized by providing a heat-developable, two-component diazotype copying material comprising a support and a light-sensitive coating on the support, the support containing at least one compound which under the action of heat pro-

2

duces a neutral or alkaline environment suitable for development in the light-sensitive coating.

The preparation of the present copying material comprises the step of impregnating a support with at least one compound, with or without additives, which under the action of heat produces a neutral or alkaline environment in the light-sensitive coating.

Materials commonly employed in diazotype techniques are suitable as support materials. It has proved advantageous to choose a support that is permeable to the compound which creates the environment in the light-sensitive mixture. Supports which fulfill this requirement are preferably paper with weights of 50 to 180 grams per square meter. These are available commercially as photocopying base papers. Transparent papers may also be used.

The compound is distributed throughout the entire support material. Under the action of heat, it creates a neutral or alkaline condition in the light-sensitive coating. Suitable compounds are those which initially exhibit no neutral or alkaline reaction and which must be heated to become converted, as by decarboxylation or fission, into products which exhibit neutral or alkaline characteristics. The following classes of compounds are suitable: monoamides or oligo-amides of organic, aliphatic, monovalent or polyvalent carboxylic acids with straight or branched chains up to approximately fifteen carbon atoms, such as acetic acid, mono-, di- and trichloroacetic acid; the diamides of carbonic acid, oxalic acid, fumaric acid or succinic acid; the amides of acids which also bear one or several hydroxyl groups in the aliphatic chain, such as the amine of malic acid, tartaric acid, citric acid, hydroxy-acetic acid, hydroxy-butyric acid, and lactic acid; and corresponding alkyl-ethers of these hydroxy carboxylic acids, such as the amide of 2-methoxy-acetic acid. Urea is preferred, particularly when used in combination with zinc chloride or trichloroacetic acid as stated below.

Additives which substantially improve the desired effect are small amounts of acids, such as trichloroacetic acid, vinylphosphonic acid and organic compounds which decompose through decarboxylation when heated to form anhydrides or ketones and thus lose their acidity. Other additives are: beta-ketonic acids, such as pyroacemic acid; beta-hydroxy acids, such as lactic acid; and malic acid. These compounds have given good results in the case of amides whose decomposition temperatures are comparatively high. Lower temperatures are afforded.

Incorporation of the substances creating the neutral or alkaline environment is preferably effected before all other process steps in the preparation of the heat-developable copying paper. Incorporation of these substances into the support material when it is not yet dry has proved particularly effective; for example, into a paper web during the paper-making process in the paper machine. By this step, the penetration of these substances into the support material is thorough. As a result, they are already present at the optimum position from which they can exert their action. Since they are not concentrated on the side which subsequently bears the light-sensitive mixture as in the usual processes, the shelf life of the copying material is substantially increased by avoidance of the premature reaction between diazo compound and coupling component.

The papers generally used have a strong sizing effect which inhibits the penetration of water and aqueous solutions. Sizings of this nature are known. This inhibitory effect of the paper's sizing does not occur in the paper-making process until the end of the drying of the paper. By incorporating the substances creating the neutral or alkaline environment before the final drying of the raw paper, very smooth complete and uniform penetration is achieved. For this operation, all stations of the paper-

making machine between web-formation and heat-drying are suitable. Suitable applicator devices are located in the final wet press and in the dry end of the paper machine. Roller applicators, such as the known sizing presses of various designs, are preferred. Other applicators include air brushes, trailing blades, and similar coating devices. The amount may vary within large or wide limits; for example, approximately one to five mole parts, preferably 1.5 to 3 mole parts theoretically necessary for the complete neutralization of the light-sensitive coating.

For special purposes, a second coating of small amounts of the substance may be made as a separate coating on the front side, although this is not necessary. The amounts of the second coating should be kept within narrow limits, such as approximately 0.1 to 0.5 mole parts for the theoretical neutralization of the other components in the light-sensitive structure.

Over this second coating, or on the paper support which has not been additionally coated, the light-sensitive mixture is coated. The mixture comprises the diazo and azo components and additives conventional in diazotype techniques.

Good results are achieved if the support material is provided with a precoat which prevents or at least inhibits penetration of the light-sensitive mixture into the support. These precoat properties must apply only to the light-sensitive mixture. The precoat must not inhibit egress of the alkaline-reacting substances or fission products out of the support.

Suitable precoat materials are: cellulose derivatives such as carboxymethyl cellulose, hydroxymethylcellulose; alginates such as sodium or ammonium alginate; organic condensates such as urea-formaldehyde or urea-glycerol resins; and many synthetic resins for the surface treatment of paper such as water-soluble resins, polyamide derivatives, alkoxy methyl/nylon, polyamine-epoxy resin, polymethyl siliconic acid sodium salt, finely-divided silicic acid of a particle size between 0.2 and 10 microns, and rice starch or oat starch. Combinations of these materials have also proved suitable. Many of them simultaneously improve contrast in the developed images.

In the case of the precoat materials, which are applied in the form of their soluble alkali metal salts or ammonium salts, care must be taken to insure adequate neutralization. This can be done by adding a suitable amount of acid to the light-sensitive preparation, by providing the pre-coated material with an intermediate coating of an acid before applying the light-sensitive coating, or by precoating with an aqueous solution of an acid and applying the substance to be neutralized as a further coating. It is also possible to acidify the precoat solution before application.

Examples of agents which have proved especially suitable for neutralization are the aqueous solutions of trichloroacetic acid, hydrochloric acid, vinyl phosphonic acid, and the like. By controlling the time interval between application of the neutralizable precoat materials and application of the neutralizing acid, or by choosing different drying temperatures after application of the precoat, it is possible to regulate the depth of penetration of the precoat material into the mass of the paper.

This effect, which is caused by the application of these precoats, aids the maintenance of the good light sensitivity during lengthy storage periods, since the light-sensitive substances are held fast near the surface of the support material. In conventional diazotype coatings, a fairly rapid decrease in light-sensitivity is observed with time.

All commonly known diazo and azo components may be used in a light-sensitive mixture. For example, 4-dimethylamino-benzene diazonium chloride, 4-diethylamino-benzene diazonium chloride, 4-N-ethyl-N-hydroxyethylamino-benzene diazonium chloride, 4-morpholino-benzene diazonium chloride, and 4-pyrrolidino-3-bromo-benzene diazonium chloride are suitable diazo components.

Suitable coupling components are: 2,3-dihydroxy-naphthalene-6-sulfonic acid; 2-hydroxy-(N-dimethyl)-naphthoic acid amide-(3); 2-hydroxy-benzotriazole (1,2); 1,3,5- resorcylic acid diethylamide; acetoacetic anilide; and 1-(N-ethylamino)-3-hydroxy-4-methyl-benzene. Mixtures of the individual components of the respective groups may also be used.

The light-sensitive mixture which is on at least one side of the support may contain additives. These additives may be classified into two groups:

(1) Additives which serve as anti-yellowing agents, wetting agents, stabilizers, and the like; that is, additives which influence the diazo and azo components in order to retain their light sensitivity, coupling properties, and their appearance as fully as possible, even after lengthy storage. Additives of this group are: thiourea, glycerol, glycol, triethanolamine hydrochloride, saponin, zinc chloride, tri-sodium naphthalene-1,3,6-trisulfonate, and the like. In this group of additives may also be included agents which influence the application properties and surface properties of the mixture with respect to its processing. These are thickening and smoothing agents, such as gelatin, carboxymethyl cellulose, and polyvinyl acetate suspensions.

(2) Additives which create a neutral or alkaline condition by the action of heat. Additives of this nature are the same as those described above for the substances in the mass of the support.

In many cases it has proved expedient to reduce the contact between the light-sensitive preparation and the substances which exert an alkaline action under heat and which are included in and incorporated into the mass of the paper by precipitating the light-sensitive diazo compound on a finely-particled support material. This is accomplished by stirring a solution of the diazo compound into a suspension of polyvinyl acetate and silica particles, then precipitating the diazo compound with polyvinyl phosphonic acid, and then coating the pre-treated papers as described.

A two-component diazotype material thus prepared is capable of being developed by heat and also may be used in the conventional copying processes. For example, in order to prepare a copy, the copying material is covered with the original to be reproduced, and exposed in contact. After separation of the original, the copying material is exposed to a brief heat treatment. This may be effected for example by irradiation with an infrared source under an infrared-absorbing material, such as a nylon sieve which has been dyed black or an infrared-absorbing paper or foil which is heat resistant up to 210° C. Treatment by pressing between two heated rollers or by passing a hot air stream over the material also yields well-developed copies. In many cases it is expedient to supply the heat by contact from the back of the copying material. A marginally sharp copy with excellent covering power of the image area is formed.

Also in the preparation of the present heat-developable material, considerable advantages result from the fact that the coating on the front side need consist only of the light-sensitive mixture by itself. In this way the constant contact between the light-sensitive mixture and the activating substance is avoided. The result is very good shelf life of the copying material.

Substantial advantages over the prior art result also when a small amount of activating substance is added to the light sensitive mixture, since this addition may be kept very small. The coating itself may be carried out in one single operation.

The copies prepared with the material according to the invention are distinguished by great sharpness. Even when the finished copies are stored for an appreciable period, the support exhibits no effect, so that legibility and contrast of the copies do not change.

The present invention is further illustrated by the following examples which are intended not to limit the scope of the inventive concept.

**5**  
**EXAMPLE 1**

A base paper suitable for diazotype techniques was impregnated in a paper making machine by means of a sizing press at the dry end with an aqueous solution of the following composition:

|               | Parts by weight |
|---------------|-----------------|
| Urea          | 10              |
| Zinc chloride | 1.33            |
| Citric acid   | 0.66            |
| Water         | 91              |

The paper was then coated on one side with a 4% aqueous solution of vinyl phosphonic acid, dried, and coated on the same side with a 1.2% aqueous solution of the sodium salt of polymethyl siliconic acid commercially available under the name Bautenschutzmittel BS/10. The paper web was dried and then coated on the same side with an aqueous solution of the following composition:

|                                                           | Parts by weight |
|-----------------------------------------------------------|-----------------|
| Trichloroacetic acid                                      | 3.2             |
| Tartaric acid                                             | 0.2             |
| 2,3 - dihydroxy-naphthalene-6-sulfonic acid (sodium salt) | 4.0             |
| Naphthalene-1,3,6-trisulfonic acid (sodium salt)          | 7.0             |
| 4-dimethylamino-benzene diazonium chloride                | 2.0             |
| Zinc chloride                                             | 1.5             |
| Urea                                                      | 1.5             |
| Gelatin                                                   | 0.09            |
| Saponin                                                   | 0.04            |
| Water                                                     | 75              |

The sensitized copying material was exposed under an original and developed by contact with heated rollers to yield contrasty, blue-colored copies having excellent shelf life, even under moist climatic conditions.

**EXAMPLE 2**

A base paper suitable for diazotype techniques was impregnated on the final wet press in the paper machine with the following solution:

|               | Parts by weight |
|---------------|-----------------|
| Urea          | 15              |
| Zinc chloride | 2               |
| Citric acid   | 1               |
| Water         | 88              |

The material thus prepared was coated on one side with the following solution:

|                                                           | Parts by weight |
|-----------------------------------------------------------|-----------------|
| Trichloroacetic acid                                      | 1.2             |
| Tartaric acid                                             | 0.2             |
| Thiourea                                                  | 4.0             |
| Naphthalene-1,3,6-trisulfonic acid (sodium salt)          | 7.0             |
| 2,3 - dihydroxy-naphthalene-6-sulfonic acid (sodium salt) | 4.0             |
| Zinc chloride                                             | 1.5             |
| 4-diethylamino-benzene diazonium chloride                 | 2.4             |
| Gelatin                                                   | 0.09            |
| Saponin                                                   | 0.04            |
| Water                                                     | 85              |

The copying material was exposed under an original and developed by heat to yield contrasty, blue-colored copies with good keeping qualities.

**EXAMPLE 3**

A suitable base paper as described in Example 1 was impregnated on the introducing or offset press of the paper machine with the following solution:

|                   | Parts by weight |
|-------------------|-----------------|
| Lactic acid amide | 30              |
| Pyroracemic acid  | 10              |
| Water             | 80              |

**6**  
The material thus obtained was coated on one side with the following solution:

|                                                                    | Parts by weight |
|--------------------------------------------------------------------|-----------------|
| Trichloroacetic acid                                               | 1.0             |
| Tartaric acid                                                      | 0.2             |
| 2,3 - dihydroxy-naphthalene-6-sulfonic acid (sodium salt)          | 4.0             |
| Thiourea                                                           | 4.0             |
| Naphthalene-1,3,6-trisulfonic acid (sodium salt)                   | 7.0             |
| Urea                                                               | 4.0             |
| 4 - N - ethyl - N - hydroxyethylamino - benzene diazonium chloride | 2.4             |
| Gelatin                                                            | 0.09            |
| Saponin                                                            | 0.04            |
| Water                                                              | 90              |

When developing by heat was effected, a blue-colored copy was obtained.

**EXAMPLE 4**

A base paper as described in Example 1 was impregnated on the sizing press of the paper machine with the following solution:

|               | Parts by weight |
|---------------|-----------------|
| Urea          | 10              |
| Zinc chloride | 1.33            |
| Citric acid   | 0.66            |
| Water         | 91              |

The material thus prepared was coated on one side with an aqueous solution of 7.5% polyvinyl phosphonic acid, dried, and coated on the same side with a 3% aqueous solution of the sodium salt of polymethyl siliconic acid commercially available under the name Bautenschutzmittel BS/10. The paper web was then dried and coated on the same side with an aqueous solution of the following composition:

|                                                                    | Parts by weight |
|--------------------------------------------------------------------|-----------------|
| Trichloroacetic acid                                               | 2.0             |
| Tartaric acid                                                      | 0.2             |
| Naphthalene-1,3,6-trisulfonic acid (sodium salt)                   | 7.0             |
| Thiourea                                                           | 4.0             |
| 2,3 - dihydroxy-naphthalene-6-sulfonic acid (sodium salt)          | 4.0             |
| Lactic acid amide                                                  | 10.0            |
| Zinc chloride                                                      | 0.5             |
| 4 - N - ethyl - N - hydroxyethylamino - benzene diazonium chloride | 2.4             |
| Gelatin                                                            | 0.09            |
| Saponin                                                            | 0.04            |
| Water                                                              | 85              |

When developing by heat was effected after exposure, a dark blue color was obtained. Copying material had excellent shelf life.

**EXAMPLE 5**

A base paper as described in Example 1 was impregnated on the introducing or off-set press of the paper-making machine with the solution described as follows:

|               | Parts by weight |
|---------------|-----------------|
| Urea          | 15              |
| Zinc chloride | 2               |
| Citric acid   | 1               |
| Water         | 88              |

The material thus obtained was coated on one side with the following solution:

|                                                           | Parts by weight |
|-----------------------------------------------------------|-----------------|
| Trichloroacetic acid                                      | 2.0             |
| Tartaric acid                                             | 0.2             |
| 2,3 - dihydroxy-naphthalene-6-sulfonic acid (sodium salt) | 4.0             |
| Naphthalene-1,3,6-trisulfonic acid (sodium salt)          | 7.0             |
| Thiourea                                                  | 4.0             |
| Tartaric acid diamide                                     | 10.0            |
| Zinc chloride                                             | 0.5             |

|                                                                    |      |
|--------------------------------------------------------------------|------|
| 4 - N - ethyl - N - hydroxyethylamino - benzene diazonium chloride | 2.4  |
| Gelatin                                                            | 0.09 |
| Saponin                                                            | 0.04 |
| Water                                                              | 80   |

When developing was effected by heat, very good blue copies of the original were obtained.

#### EXAMPLE 6

A base paper as described in Example 1 was impregnated on the introducing or off-set press of the paper-making machine with the following solution:

| Parts by weight      |    |
|----------------------|----|
| Urea                 | 15 |
| Trichloroacetic acid | 3  |
| Water                | 85 |

The material thus obtained was then coated on one side with a 5% aqueous solution to a polyamide-epoxide resin commercially available under the name Nadavin. After drying, coating was carried out with a solution of the following composition:

| Parts by weight                                         |      |
|---------------------------------------------------------|------|
| Trichloroacetic acid                                    | 1.0  |
| Tartaric acid                                           | 0.2  |
| 2,3-dihydroxy-naphthalene-6-sulfonic acid (sodium salt) | 4.0  |
| Thiourea                                                | 4.0  |
| Naphthalene-1,3,6-trisulfonic acid (sodium salt)        | 7.0  |
| Urea                                                    | 2.5  |
| Zinc chloride                                           | 0.5  |
| 4-dimethylamino-benzene diazonium chloride              | 2.4  |
| Gelatin                                                 | 0.09 |
| Saponin                                                 | 0.04 |
| Water                                                   | 80   |

After exposure, there was obtained by heating, a very contrasty, blue copy of the original.

#### EXAMPLE 7

A base paper as described in Example 1 was impregnated on the final wet press of the paper machine with the following solution:

| Parts by weight |    |
|-----------------|----|
| Urea            | 15 |
| Zinc chloride   | 2  |
| Citric acid     | 1  |
| Water           | 88 |

The material thus prepared was coated on one side with an aqueous solution of 3% of the sodium salt of polymethyl silicone acid commercially available under the name Bautenschutzmittel BS/10 and 1% sodium alginate. After drying, the following solution was applied to the same side of the paper:

| Parts by weight                                         |      |
|---------------------------------------------------------|------|
| Tartaric acid                                           | 1.5  |
| 2,3-dihydroxy-naphthalene-6-sulfonic acid (sodium salt) | 4.0  |
| Thiourea                                                | 4.0  |
| Naphthalene-1,3,6-trisulfonic acid (sodium salt)        | 4.0  |
| 4-dimethylamino-benzene diazonium chloride              | 2.4  |
| Gelatin                                                 | 0.09 |
| Saponin                                                 | 0.04 |
| Urea                                                    | 5.0  |
| Water                                                   | 80   |

After exposure, there was obtained by heating, a good, dark blue copy of the original.

#### EXAMPLE 8

A base paper as described in Example 1 was impregnated in the paper machine by means of a sizing press inside the dry end with an aqueous solution of the following composition:

| Parts by weight                                      |      |
|------------------------------------------------------|------|
| Urea                                                 | 10.0 |
| Urea-glycerol resin prepared by melting together and |      |

| Parts by weight                                                  |     |
|------------------------------------------------------------------|-----|
| heating for one hour at 120° C. equal parts of urea and glycerol | 8.5 |
| Water                                                            | 82  |

5 The material thus obtained was coated on one side with the following solution:

| Parts by weight                                         |      |
|---------------------------------------------------------|------|
| Tartaric acid                                           | 0.2  |
| 2,3-dihydroxy-naphthalene-6-sulfonic acid (sodium salt) | 4.0  |
| Thiourea                                                | 4.0  |
| Naphthalene-1,3,6-trisulfonic acid (sodium salt)        | 4.0  |
| 4-dimethylamino-benzene diazonium chloride              | 1.7  |
| Saponin                                                 | 5.0  |
| Gelatin                                                 | 0.09 |
| Water                                                   | 85   |

After exposure, when developing by heat was effected, a blue copy of the original was obtained.

#### EXAMPLE 9

A transparent base paper suitable for diazotype techniques was impregnated in the paper machine by means of an air brush applicator inside the dry end with the following solution:

| Parts by weight |      |
|-----------------|------|
| Urea            | 10   |
| Zinc chloride   | 1.33 |
| Citric acid     | 0.66 |
| Water           | 91   |

The material thus obtained was coated on one side with a solution of 7.5% methoxymethyl poly- $\epsilon$ -caprolactam in 70% methanol and, after drying, the following solution was applied to the same side of the paper:

| Parts by weight                                         |      |
|---------------------------------------------------------|------|
| Trichloroacetic acid                                    | 3.2  |
| Tartaric acid                                           | 0.2  |
| 2,3-dihydroxy naphthalene-6-sulfonic acid (sodium salt) | 4.0  |
| Thiourea                                                | 4.0  |
| Naphthalene-1,3,6-trisulfonic acid (sodium salt)        | 7.0  |
| Urea                                                    | 10.0 |
| 4-dimethylamino-benzene diazonium chloride              | 2.0  |
| Zinc chloride                                           | 1.5  |
| Gelatin                                                 | 0.09 |
| Saponin                                                 | 0.04 |
| Water                                                   | 75   |

After exposure, when developing by heat was effected, a blue copy of the original was obtained.

#### EXAMPLE 10

A base paper was treated on the sizing press in the paper machine with the following solution:

| Parts by weight |    |
|-----------------|----|
| Urea            | 15 |
| Zinc chloride   | 2  |
| Citric acid     | 1  |
| Water           | 88 |

60 The material thus obtained was coated with an aqueous suspension prepared in the following manner:

| Parts by weight                                                                                                                                                                                   |  |
|---------------------------------------------------------------------------------------------------------------------------------------------------------------------------------------------------|--|
| 4 parts by weight of a finely-particled silicic acid with a grain size distribution lying mainly between 1 and 10 microns                                                                         |  |
| were suspended in 70 parts by volume of a 1.5% aqueous solution of the sodium salt of a polymethyl silicic acid commercially available under the name Bautenschutzmittel BS/10.                   |  |
| 20 parts by volume of a 20% by weight suspension of a polyvinyl acetate copolymer commercially available under the designation Mowilith DMC No. 2 were then added.                                |  |
| To the suspension thus obtained there was added, gradually and with vigorous stirring, 10 parts by volume of a 10% aqueous solution of monomeric vinylphosphonic acid, and the whole then stirred |  |
| 75 briskly for an hour.                                                                                                                                                                           |  |

After drying, the pre-treated paper was coated on the same side with a solution of the following composition:

|                                                         | Parts by weight |
|---------------------------------------------------------|-----------------|
| Trichloroacetic acid                                    | 0.2             |
| Tartaric acid                                           | 0.2             |
| Naphthalene 1,3,6-trisulfonic acid (sodium salt)        | 7.0             |
| Thiourea                                                | 4.0             |
| 2,3-dihydroxy-naphthalene-6-sulfonic acid (sodium salt) | 4.0             |
| Triethanolamine hydrochloride                           | 4.0             |
| Urea                                                    | 5.0             |
| Zinc chloride                                           | 0.5             |
| Gelatin                                                 | 0.09            |
| Saponin                                                 | 0.04            |
| 4-dimethylamino-benzene diazonium chloride              | 2.0             |
| Water                                                   | 90              |

The paper thus prepared was distinguished by particularly good shelf life and high contrast. After exposure under a transparent original, it was developed by heating up to 160° to 170° C. A good blue-colored positive copy of the original was obtained.

It is evident that the described examples are capable of many variations and modifications. All such variations and modifications are to be included within the scope of the present invention.

What is claimed is:

1. A heat-developable reproduction material which comprises:
  - a paper support impregnated in the paper-making process with a mixture of urea and urea-glycerol resin; and
  - a light-sensitive diazo coating comprising a diazonium compound, an azo coupling component and an acid stabilizer on at least one side of the support, said coating being developable by the action of heat on the mixture of urea and urea-glycerol resin.
2. A heat-developable reproduction material which comprises:
  - a paper support impregnated in the paper-making process with a mixture of lactic acid amide and pyroracemic acid, which mixture, when heated, is activated to generate an alkaline environment; and
  - a light-sensitive diazo coating comprising a diazonium compound, an azo coupling component and an acid stabilizer on at least one side of the support, said coating containing urea and being developable by the action of heat on the mixture of lactic acid amide and pyroracemic acid and the urea.
3. A heat-developable reproduction material which comprises:
  - a paper support impregnated in the paper-making process with urea; and
  - a light-sensitive diazo coating comprising a diazonium compound, an azo coupling component and an acid stabilizer on at least one side of the support, said coating containing tartaric acid amide and being developable by the action of heat on the urea and the tartaric acid amide.
4. A heat-developable reproduction material which comprises:
  - a paper support impregnated in the paper-making process with urea;
  - a layer of polymethyl siliconic acid sodium salt and sodium alginate; and
  - a light-sensitive diazo coating comprising a diazonium compound, an azo coupling component and an acid stabilizer on the layer, said coating containing urea and being developable by the action of heat of the urea.

5. A heat-developable reproduction material which comprises:

a transparent paper support impregnated in the paper-making process with urea;

a layer of methoxy methyl poly- $\epsilon$ -caprolactam; and

a light-sensitive diazo coating comprising a diazonium compound, an azo coupling component and an acid stabilizer on the layer, said coating containing urea and being developable by the action of heat on the urea.

6. A heat-developable reproduction material which comprises:

a paper support impregnated in the paper-making process with urea;

a layer of silicic acid, polymethyl siliconic acid sodium salt, and polyvinyl acetate; and

a light-sensitive diazo coating comprising a diazonium compound, an azo coupling component and an acid stabilizer on the layer, said coating containing urea and being developable by the action of heat on the urea.

7. A heat-developable reproduction material which comprises:

a paper support impregnated in the paper-making process with urea;

a first layer of vinyl phosphonic acid coated on at least one side of the support;

a second layer of polymethyl siliconic acid sodium salt coated on the first layer; and

a light-sensitive diazo coating comprising a diazonium compound, an azo coupling component and an acid stabilizer on the second layer, said coating containing urea and being developable by the action of heat on the urea.

8. A heat-developable reproduction material which comprises:

a paper support impregnated in the paper-making process with urea;

a first layer of polyvinyl phosphonic acid coated on at least one side of the support;

a second layer of polymethyl siliconic acid sodium salt coated on the first layer; and

a light-sensitive diazo coating comprising a diazonium compound, an azo coupling component and an acid stabilizer on the second layer, said coating containing lactic acid amide and being developable by the action of heat on the urea and the lactic acid amide.

#### References Cited

##### UNITED STATES PATENTS

|           |         |                |          |
|-----------|---------|----------------|----------|
| 2,617,727 | 11/1952 | Slifkin        | 96—75    |
| 3,159,487 | 12/1964 | Krieger et al. | 96—91 XR |
| 3,169,067 | 2/1965  | Berman et al.  | 96—91    |
| 3,312,551 | 4/1967  | Sus            | 96—49 XR |
| 3,076,707 | 2/1963  | Lawton et al.  | 96—49 XR |
| 3,255,007 | 6/1966  | Kosar          | 96—91 XR |

##### FOREIGN PATENTS

|           |         |                |
|-----------|---------|----------------|
| 12,096    | 7/1963  | Japan.         |
| 597,615   | 5/1960  | Canada.        |
| 907,724   | 10/1962 | Great Britain. |
| 909,491   | 10/1962 | Great Britain. |
| 931,668   | 7/1963  | Great Britain. |
| 1,249,913 | 11/1960 | France.        |

NORMAN G. TORCHIN, Primary Examiner.

C. BOWERS, Assistant Examiner.

U.S. Cl. X.R.